

## UNITED STATES PATENT OFFICE

2,413,928

## HEAT TREATMENT FOR MAGNESIUM ALLOYS

James F. Simpson, Old Greenwich, Conn., assignor to American Cyanamid Company, New York, N. Y., a corporation of Maine

No Drawing. Application October 14, 1944.  
Serial No. 558,741

11 Claims. (Cl. 148—21.3)

1

The present invention relates to the heat treatment of magnesium base alloys and to a fused bath therefor.

Heretofore magnesium base alloys have only been heat treated to improve their mechanical properties in a circulating gas furnace. Treatment therein is hazardous in that there is danger of fire by reason of the material treated. It has been proposed to introduce sulfur dioxide into the atmosphere of the furnace to prevent burning of the magnesium at treating temperatures but leakage of  $\text{SO}_2$  is a nuisance and health hazard.

The principal object of the invention is to provide a method and means of heat treating magnesium base alloys which will produce mechanical properties in the alloys treated as good or better than those now obtained by treatment in the usual circulating air furnace, which will have no fire hazard, which will be inert chemically to the alloy, which will be cheap, and otherwise desirable.

To this end the invention contemplates the heat treating of magnesium base alloys in a molten bath comprising KCNO in predominant quantity. By this expression is meant KCNO alone or in admixture with minor quantities of such salts as KCl, NaCl, KCN, NaCN, NaCNO,  $\text{MgCl}_2$ ,  $\text{K}_2\text{CO}_3$ , or the like. The exact composition of the bath whether of KCNO alone or in admixture with one or more of the above salts will in some measure depend upon the temperature required for the desired heat treatment as obviously no treatment in such baths may be had prior to their melting point which varies considerably. For instance, baths in which magnesium base alloys may be satisfactorily heat treated are given below together with their melting points:

|    | Bath composition                                                          | Melting point |
|----|---------------------------------------------------------------------------|---------------|
| 1. | KCNO 100%                                                                 | 558-590       |
| 2. | { KCNO 87%<br>KCl 13%                                                     | 545-550       |
| 3. | { KCNO 87%<br>NaCN 13%                                                    | 525           |
| 4. | { KCNO 86%<br>KCN 14%                                                     | 540           |
| 5. | { KCNO 90%<br>NaCl 10%                                                    | 550           |
| 6. | { KCNO 88%<br>NaCNO 12%                                                   | 580           |
| 7. | { KCNO 88%<br>NaCN 4%                                                     | 580           |
| 8. | { KCNO 8%                                                                 |               |
| 9. | { KCNO 73%<br>MgCl <sub>2</sub> 15%<br>K <sub>2</sub> CO <sub>3</sub> 12% | 580           |

While the above compositions represent substantially eutectic mixtures the proportions may be reasonably varied when slightly higher temperatures are desired. Such baths may be used at temperatures varying from their melting point

5

up to a temperature just short of substantial decomposition. While the temperature and time of treatment will vary slightly dependent upon the actual composition and mass of the magnesium base alloy yet this is a minor variation as in all cases it has been found that the temperature and time of treatment is substantially that now used for the same alloys in circulating air furnaces.

The usual solution heat treatment of magnesium base alloys in air type heating furnaces involves generally heating the work to from 630-760° F., holding the piece at one or more places in the temperature scale for from 5-20 hours followed by air quenching. The same conditions have been found to be satisfactory in the heat treatment of such alloys in fused baths of the present invention.

The following alloys and their treatment are typical of practice under the present invention.

The specifications of mechanical properties for a cast magnesium base alloy referred to herein as alloy A and consisting of:

|                                           |             |
|-------------------------------------------|-------------|
| Aluminum                                  | 5.3-6.7     |
| Zinc                                      | 2.5-3.5     |
| 25 Manganese                              | .15 maximum |
| Silicon                                   | .5 maximum  |
| Copper                                    | .05 maximum |
| Metals other than the above and magnesium | .3 maximum  |
| 30 Magnesium                              | Remainder   |

are as follows:

## Mechanical properties

|                            | Condition | As cast | Solution treated | Solution and precipitation treated |
|----------------------------|-----------|---------|------------------|------------------------------------|
| 40 Yield strength          | p. s. i.  | 10,000  | 10,000           | 16,000                             |
| Tensile strength           | do        | 24,000  | 32,000           | 34,000                             |
| Elongation, per cent in 2" | 4         | 6       | 2                |                                    |

The prevalent recommended solution heat treating and subsequent precipitation cycles used in conventional circulating air type heat treating furnace are as follows:

## Solution treatment

1. Hold at 630°-640° F. for five hours;
2. Raise temperature to 710°-720° F. and hold for 13 hours;
3. Air quench.

## Precipitation treatment

4. Hold at 350° F. for 16 hours;
5. Air cool.

Test bars of alloy A were solution heat treated in a bath comprising substantially 87% potassium cyanate and substantially 13% potassium chloride (a substantially eutectic mixture) and

duplicate bars treated in a conventional air furnace according to the above prevalent heat treating cycles. The solution heat treated bars were precipitation heat treated in an ordinary air oven with no chemical correctives in the atmosphere. The mechanical properties of test bars of alloy A so treated are indicated below:

Table I  
ALLOY A SOLUTION AND PRECIPITATION TREATED

| Bar No.               | Treatment   | Yield strength, p. s. i. | Tensile strength, p. s. i. | Permanent elongation, percent in 2" lengths | Hardness, Brinell |
|-----------------------|-------------|--------------------------|----------------------------|---------------------------------------------|-------------------|
| Specifications.       |             | 16,000 min.              | 34,000 min.                | 3                                           | 65 min.           |
| CH 212                | Bath        | 19,200                   | 41,200                     | 6.5                                         | 68                |
| CH 212                | Air furnace | 18,750                   | 36,550                     | 4                                           | 68                |
| CH 242                | Bath        | 19,850                   | 41,650                     | 6.5                                         | 67                |
| CH 242                | Air furnace | 19,000                   | 37,000                     | 5                                           | 69                |
| CH 251A               | Bath        | 18,600                   | 41,400                     | 7                                           | 68                |
| CH 251B               | do          | 19,000                   | 39,000                     | 5.5                                         | 68                |
| CH 251                | Air furnace | 18,240                   | 37,920                     | 4                                           | 67                |
| CH 252                | Bath        | 19,500                   | 41,650                     | 5.5                                         | 70                |
| CH 252                | Air furnace | 18,820                   | 36,230                     | 4                                           | 71                |
| CH 271                | Bath        | 19,500                   | 41,100                     | 6                                           | 67                |
| CH 271                | Air furnace | 19,230                   | 34,810                     | 3.5                                         | 68                |
| CH 272                | Bath        | 20,170                   | 36,650                     | 4                                           | 68                |
| CH 272                | Air furnace | 17,220                   | 33,460                     | 3                                           | 70                |
| CH 282                | Bath        | 22,220                   | 38,750                     | 4                                           | 72                |
| CH 282                | Air furnace | 16,800                   | 35,470                     | 4                                           | 74                |
| SOLUTION TREATED ONLY |             |                          |                            |                                             |                   |
| Specifications.       |             | 10,000 min.              | 32,000 min.                | 6                                           |                   |
| CH 302                | Bath        | 17,975                   | 38,150                     | 11.5                                        |                   |
| CH 312A               | do          | 13,225                   | 37,000                     | 10.5                                        |                   |
| CH 312B               | do          | 13,475                   | 38,225                     | 12.5                                        |                   |
| 11                    | do          | 13,350                   | 35,900                     | 9.5                                         |                   |
| 2                     | do          | 14,175                   | 37,050                     | 10                                          |                   |
| 22                    | do          | 14,125                   | 37,350                     | 10.5                                        |                   |

<sup>1</sup> Denotes edge inclusion.

Another slightly different magnesium base alloy hereinafter referred to as alloy B, composed as follows:

|                                              |             |
|----------------------------------------------|-------------|
| Aluminum                                     | 8.3-9.7     |
| Zinc                                         | 1.7-2.5     |
| Manganese                                    | 1.0 maximum |
| Silicon                                      | .50 maximum |
| Copper                                       | .05 maximum |
| Nickel                                       | .03 maximum |
| Materials other than the above and magnesium | .30 maximum |
| Magnesium                                    | Remainder   |

was heated in a bath of the present invention according to the prevalent heat treating cycle currently used in the conventional circulating air type furnace, as follows:

#### Solution treatment

1. Heat to and hold at  $760 \pm 5^{\circ}$  F. for 20 hours;
2. Air cool.

#### Precipitation treatment

3. Heat to  $350^{\circ}$  F. and hold for 12 hours;
4. Air cool.

The results of the treatment of samples of alloy B according to the above is shown below as compared with the standard specification of mechan-

ical characteristics for the conventionally treated alloy:

Table II

5 ALLOY B SOLUTION AND PRECIPITATION TREATED

| Bar No.        | Treatment | Yield strength, p. s. i. | Tensile strength, p. s. i. | Permanent elongation, per cent in 2" lengths |
|----------------|-----------|--------------------------|----------------------------|----------------------------------------------|
| Specifications |           | 18,000                   | 34,000                     | 1                                            |
| B. C. 141      | Bath      | 23,800                   | 35,900                     | 1                                            |
| B. C. 151      | do        | 24,000                   | 36,250                     | 1                                            |
| B. C. 152      | do        | 23,450                   | 40,600                     | 1.5                                          |
| C. C. 181      | do        | 26,100                   | 35,200                     | 1                                            |
| C. C. 182      | do        | 25,900                   | 34,800                     | 1                                            |
| C. C. 201      | do        | 23,750                   | 36,850                     | 1                                            |
| C. C. 211      | do        | 23,700                   | 37,700                     | 1                                            |

SOLUTION TREATED ONLY

| Specifications | Treatment | Yield strength, p. s. i. | Tensile strength, p. s. i. | Permanent elongation, per cent in 2" lengths |
|----------------|-----------|--------------------------|----------------------------|----------------------------------------------|
| C. C. 181      | Bath      | 15,900                   | 33,500                     | 6                                            |

In all cases of treated alloys A and B neither the solution heat treatment nor the precipitation treatment detrimentally affected the mechanical properties nor the surface condition of the alloys.

It was found that such baths actually act as an insulator against the burning of the magnesium base alloys even when severely overheated.

Treatment in a fused salt bath is particularly advantageous over air furnace heating in that the work piece can be suspended from wires, thus eliminating the necessity of heating the non-productive portion of the charge such as trucks, baskets and the like required in the standard air type heating furnaces.

Any bath material adhering to the work after treatment may be readily washed off in water.

Baths of this type lose only a very small part of the content through vaporization as it has been found that only 2.4% by weight was lost through such cause after 40 hours of continuous operation at  $750^{\circ}$  F. In addition, any slow increments in decomposition products of the bath up to a concentration of more than 30% is completely soluble in the bath at the treating temperature.

This minimizes sludge formation and consequent detrimental effects on the heating pot and work piece due to localized overheating. The presence of the decomposition product or products has no apparent effect on either the mechanical properties nor the surface condition of the alloys treated.

In all cases where the treated alloys were etched for five seconds in a standard glycol etchant it has been found that there was vast improvement in distribution of the component parts of the alloy as compared with an untreated piece.

While the invention has been described with particular reference to specific embodiments, yet it is to be understood that the invention is not to be limited thereto, but is to be construed broadly and restricted solely by the scope of the appended claims.

#### What is claimed:

1. A method of heat treating a magnesium base alloy work piece which includes the steps of immersing the same in a molten bath predominately of KCNO at a solution heat treating temperature until the distribution of the alloy components has been improved, removing the work piece from the bath and air quenching the same.

2. A method of heat treating a magnesium base alloy work piece which includes the steps of immersing the same in a molten bath predominately of KCNO and also containing KCl at a solution heat treating temperature until the distribution of the alloy components has been improved, removing the work piece from the bath and air quenching the same.

3. The method of claim 2 in which the bath contains substantially 87% KCNO and substantially 13% KCl.

4. The method of claim 2 in which the bath temperature is from 630°-640° F. and the time is substantially 5 hours.

5. The method of claim 2 in which the bath temperature is from 630-640° F. and the time is substantially 5 hours, and thereafter raising the bath temperature to from 710-720° F., holding that temperature for substantially 13 hours, removing the work piece from the bath and air quenching.

6. The method of claim 2 in which the bath temperature is from 630-640° F. and the time is substantially 5 hours, and thereafter raising the bath temperature to from 710-720° F., holding that temperature for substantially 13 hours, removing the work piece and air quenching, heating the work piece in air to substantially 350° F., holding the same for substantially 16 hours, removing the work piece and air quenching.

7. A method of heat treating a magnesium base alloy work piece which includes the steps of immersing the same in a molten bath containing substantially 87% KCNO and substantially 13% KCl at from 710-720° F. for 13 hours, removing the work piece, air quenching, heating the work piece in air for substantially 16 hours at substantially 350° F., removing the work piece and air quenching.

8. The method of claim 6 in which the alloy is of substantially the following composition:

|                                           |             |
|-------------------------------------------|-------------|
| Aluminum                                  | 5.3 - 6.7   |
| Zinc                                      | 2.5 - 3.5   |
| 5 Manganese                               | .15 maximum |
| Silicon                                   | .5 maximum  |
| Copper                                    | .05 maximum |
| Metals other than the above and magnesium | .3 maximum  |
| 10 Magnesium                              | Remainder   |

9. The method of claim 3 in which the heating is carried out at substantially 760° F. for substantially 20 hours.

15 10. The method of claim 3 in which the piece is solution treated at substantially 760° F. for about 20 hours, removing the work piece, air cooling, and heating the work piece to substantially 350° F. for about 12 hours and removing the work piece and air quenching.

20 11. The method of claim 3 in which the piece is an alloy of substantially the following composition:

|           |             |
|-----------|-------------|
| Aluminum  | 8.3 - 9.7   |
| 25 Zinc   | 1.7 - 2.5   |
| Manganese | 1.0 maximum |
| Silicon   | .50 maximum |
| Copper    | .05 maximum |
| Nickel    | .03 maximum |

30 30 Materials other than the above and magnesium .30 maximum Magnesium Remainder

and is solution treated at substantially 760° F. for about 20 hours, removed, air cooled and then heated for about 12 hours, at substantially 350° F. in air, removing the work piece and air quenching.

JAMES F. SIMPSON.